

1

2,804,073

## FLUID SURGICAL DRESSING

William F. Gallienne, Springfield, and William E. Le May and Louis Pereny, Dayton, Ohio, assignors to Protective Treatments, Inc., Dayton, Ohio, a corporation of Ohio

No Drawing. Application January 26, 1953,  
Serial No. 333,366

6 Claims. (Cl. 128—156)

This invention relates to a surgical dressing for wounds, burns and the like and, more particularly, to a transparent releasably adhesive dressing adapted to be applied as a liquid or spray.

According to this invention a surgical dressing is provided in the form of a tough, elastic, transparent film with mildly bacteriostatic properties. The film is non toxic, chemically inert, insoluble in body fluids; it is resistant to water while being sufficiently permeable to moisture vapor to prevent formation of blisters thereunder. The transparent film dressing includes an adhesive component providing controllable adhesion such that it adheres to normal skin sufficiently to anchor the film firmly yet be readily peelable for removal, and has little if any adhesion to raw flesh of an open wound or burned area or to newly formed skin beneath the dressing. Essentially this dressing is stable, impermeable to coliform group organisms, sterile, and adapted to be applied by wiping on, brushing and in the form of a spray. It is of such character that laymen without medical training can apply the dressing so as to form an artificial skin over a wound or burn to stabilize the injured area and protect it until further medical treatment is obtained.

It is accordingly an object of this invention to provide as a new composition a sprayable liquid to be applied to wounds, burns, and the like to form thereover a non-toxic, sterile, releasably adhesive, transparent, water resistant, bacteriostatic, semipermeable film.

A further object of this invention is to provide in liquid composition a film forming component, a controlled adhesion producer, a plasticizer, and a bacteriostatic agent in a nontoxic vehicle for application to form a dressing of the character described.

Still another object of this invention is to provide a liquid composition of the character described including a controlled adhesion producing component, separate from the film forming component, which forms releasable adhesion to normal skin without adhering to the injured area.

Another object of this invention is to provide a liquid composition of the character described which upon drying forms a tough, elastic film over a wound sufficiently permeable to permit outward moisture vapor transmission from the wound while being substantially impermeable to the inward passage of infection promoting organisms.

Still a further object of this invention is to provide a liquid composition of the character described which upon drying produces over a wound a transparent elastic film adherent to normal skin, nonadherent to raw flesh, and peelable from normal skin without softening or other treatment.

Still another object of this invention is to provide a liquid composition of the character described for application to human skin and injured areas thereof, with the composition having a toxicity or allergic reactivity level at least as low as conventional surgical dressing adhesives, and being substantially free of medication.

2

A further object of this invention is to provide a solvent or dispersion vehicle adapted to admit of application of a tough, elastic, transparent film dressing of the character described and of low smarting, nonirritating and nontoxic physiological effect on exposed tissue in open wounds, burns, and the like.

Other objects and advantages of this invention will be apparent from the following description and the appended claims.

10 In the treatment of many injuries, the immediate application of a sterile dressing may be of controlling importance particularly to prevent loss of body fluids and continued exposure of the injured area to bacteria and other sources of infection. For example, in burns where 15 large areas of skin are destroyed, the loss of serum from the burned area is an important source of shock and perhaps fatality. Especially in instances where large numbers of people may be severely injured is it important to have available emergency treatment adapted for safe application by essentially untrained personnel. Considering, for example, a situation where a human being has 20 suffered 50% body burns, it has been found that it may require a trained doctor and nurse over an hour to apply a standard ointment and pressure bandage consisting of several pounds of ointment and perhaps 120 yards of bandage to provide emergency treatment. By contrast, 25 the same burned area could be satisfactorily treated in about five minutes by two laymen using but four spray containers of a sprayable dressing embodying this invention. Also the desirability of a transparent surgical dressing is advantageous for the observation of healing of a wound or burn without inevitable trauma and exposure to infection occasioned by repeated removals of the dressing to inspect the wound.

30 According to this invention a sprayable plastic composition is produced which will form upon application a transparent film over the injured area. The film, in addition to being transparent, is water-resistant and insoluble in body fluids. At the same time it is sufficiently semi- 35 permeable to admit of the outward penetration of water vapor to preclude the formation of a water blister under the dressing when perspiration and/or other body fluids collect. Such semipermeability does not destroy the continuity of the film nor render it permeable to the inward 40 passage of objectionable bacteria, and is essentially a controlled degree of moisture-vapor transmission as opposed to mechanical porosity.

In addition to being tough and sufficiently elastic to 45 protect the wound and accommodate body movement, the film is also, when applied sufficiently adhesive to normal skin surrounding the injured area to maintain itself in position, yet readily removable by peeling without softening or other treatment. The film has, however, very limited if any adhesiveness for the exposed raw flesh of 50 the injured area, and is of such character as to avoid adhesion to newly formed skin growing under the dressing. That is, compositions according to this invention exhibit 55 selective adhesion to dry instead of wet skin or flesh.

Both the final dressing and its sprayable liquid original 60 composition are relatively nontoxic to either normal skin or the injured area and exhibit low allergic reactivity. With the preferred compositions described below, the allergic reactivity level is less than that of medically accepted commercial surgical adhesive tape. The solvent or vehicle utilized preferably has a relatively low smarting 65 level and is of such character as will not promote flow of blood or other body fluids.

For application of the sprayable dressing by essentially untrained personnel, it includes substantially no medication, although it preferably includes components to maintain sterility or a bacteriostatic condition—i. e., it stabilizes 70 and maintains existing conditions in the injured area

preceding or following suitable professional medical treatment. The original liquid composition before application is substantially stable and nonoxidizing for convenient storage and maintains its own sterility and/or includes components which discourage the existence of obnoxious bacteria. Because of the selective or controlled adhesion to dry or healthy skin without adhesion to raw flesh and because of the insolubility of film components in body fluids there is substantially no transfer of film components into the wound or to newly formed skin beneath the bandage.

A sprayable surgical dressing having the attributes noted has been produced according to this invention by the combination of a film former, an adhesion producer, a plasticizer, and a bacteriostatic agent, which components are admixed to form, with a suitable vehicle, a liquid solution or emulsion. In addition to the dry film properties noted above, the liquid compositions according to this invention are stable to exposure to temperatures ranging from  $-65^{\circ}$  F. to  $+165^{\circ}$  F. in storage and are usable at temperatures ranging from  $20^{\circ}$  F. up to  $130^{\circ}$  F. In the form of an aqueous emulsion, the smarting level in contact with raw flesh may be lower than when volatile organic solvents are used, although a solution of the liquid compositions may be readily post-emulsified to decrease the smarting effect if desired. When volatile solvents are used, the drying time of the film can be easily controlled, and is usually of the order of five minutes, while with application of the dressing in the form of a water emulsion, this time may be increased if desired to about fifteen minutes or more.

Considering a solution type liquid composition to give upon drying a plastic dressing embodying this invention, the film former may be present in the proportion of about 100 parts by weight; the adhesion producer in from 5 to 80 parts by weight with approximately 50 parts being preferred; the plasticizer in up to 80 parts by weight with approximately 50 being preferred; and the bacteriostatic agent in up to 2 parts by weight with approximately .25 being preferred. The bacteriostatic agent may be present as a part of the adhesion producing component. Sufficient nontoxic and volatile solvent is incorporated to produce the desired consistency with about 800 parts being preferred.

Such a composition is packed in metal containers or so-called "aerosol" spray-type containers accompanied by suitable well-known spray propellants such as halogenated-aliphatic type or compressed gaseous type propellants if application is desired by aerosol spray. It may also be applied by compressed gas spray, brushing, flowing, wiping on, or dipping.

The film forming component may be of the class consisting of vinyl polymers (including vinyl chloride-vinylidene component copolymers, vinyl chloride-vinyl acetate copolymers and carboxylated or hydroxylated modifications of such copolymers, vinyl chloride-butadiene polymers, vinyl butyral polymers, vinyl acetate polymers, etc.), polyacrylic and polymethacrylic esters and polymers, cellulose acetate butyrate, ethyl cellulose, and compatible combinations thereof. The adhesion producing component may be one or compatible combinations of such resins as glycerol phthalate, abietic acid-glycerol and organic acid and/or phenol modifications of such abietic acid glycerol, amine-aldehyde resins, and resins containing maleic anhydride or phenols (including cresols). The plasticizer may be one or a combination of such monomeric substances as dioctyl phthalate, butyl phthalate butyl glycolate, di-2(ethyl-hexyl) azelate, acetylated castor oil, phthalic anhydride-vegetable oil derivatives, tricresyl phosphate, o- and p-toluene sulfonamides; or polymeric substances such as chlorinated paraffin, cumarone-indene, sebacic acid polymers, treated raw oiticica and other vegetable oils (treated to produce compatibility with film formers). The bacteriostatic agent may satisfactorily be maleic anhydride (as included, for example, in the ad-

hesive component), phenols (including cresols), and compatible physiologically appropriate mercury compounds.

Satisfactory volatile solvents for the above include one or a combination of such solvents as organic esters (e. g., 5 ethyl acetate), ketones (e. g. acetone), organic ethers or oxides (e. g. ethylene oxide), aromatic hydrocarbons (e. g., toluene), or chlorinated aliphatic hydrocarbons (e. g., methylene chloride). The solvent component is chosen to produce the desired drying rate and viscosity 10 of liquid composition with regard to method of application, ease of storage, traumatic smarting effect, etc. As noted above, such a solution may be post-emulsified by the addition of appropriate emulsifying agents, anti-foaming agents, and water.

15 A satisfactory method of preparation of the composition includes adding the film former slowly to the solvent with agitation in a suitable covered container taking care to avoid agglomeration. The remaining ingredients are 20 added upon the complete solution of the film former and agitation is continued until all ingredients are dissolved. After suitable filtration to remove any suspended foreign matter, the liquid composition is packed into aerosol spray containers at approximately  $0^{\circ}$  F. in known manner, or otherwise packaged as desired.

25 As a specific example of a solution type composition embodying this invention, satisfactory results have been experienced with a combination of:

#### Example 1

|                                                         | Parts by weight |
|---------------------------------------------------------|-----------------|
| 30 Hydroxylated vinyl acetate-vinyl chloride co-polymer | 100             |
| Maleic anhydride modified, glycerol-abietic-acid resin  | 50              |
| 35 Sebacic acid co-polymer type plasticizer             | 50              |
| Ethyl acetate                                           | 600             |
| CP acetone                                              | 200             |

#### Example 2

|                                             |     |
|---------------------------------------------|-----|
| 40 N-butyl methacrylate polymer             | 120 |
| Butyl phthalyl butyl glycolate              | 30  |
| Phenol-modified glycerol-abietic-acid resin | 50  |
| Ethyl acetate                               | 800 |

#### Example 3

|                                                        |     |
|--------------------------------------------------------|-----|
| 45 Ethyl cellulose                                     | 80  |
| Di-octyl phthalate                                     | 80  |
| Maleic anhydride modified, glycerol-abietic-acid resin | 40  |
| Ethyl acetate                                          | 800 |

#### Example 4

|                                                                          |     |
|--------------------------------------------------------------------------|-----|
| 50 Vinyl chloride-vinyl acetate resin VAGH                               | 100 |
| Paraplex G-50 (proprietary epoxidized-oil type plasticizer)              | 50  |
| 55 Amberlac D-96 (maleic anhydride modified glycerol-abietic-acid resin) | 50  |
| Ethyl acetate                                                            | 800 |

60 In the above examples the particular solvent was chosen for rate of drying, although other solvent blends may be used where necessary to slow up drying or to meet special requirements. It has been found, for example, that volatile chlorinated solvents have no deleterious effect on dried film properties when added to the liquid composition in the range of one volume of composition to two volumes of solvent. The concentration of plasticizer may also be varied to produce the desired flexibility or softness indicated by the requirements of use. The above noted maleic anhydride modified resin includes the bacteriostatic component because of its fungistatic and bacteriostatic properties and the proportions may be varied to a limited extent to produce the desired hardness, adhesiveness and flexibility suited for a particular application.

70 A suitable composition of the aqueous emulsion type embodying this invention includes a film forming com-

ponent in the form of a latex or emulsion on a 50% nonvolatile basis in the range of approximately 200 parts by weight, a separate adhesion producer up to 80 parts by weight with 5 parts being preferred, a plasticizer up to 80 parts by weight with 1 part being preferred, a bacteriostatic agent up to 2 parts by weight with .25 being preferred (may be included with adhesion producer), and volatile solvents up to 20 parts by weight with 5 being preferred. The above composition is emulsified with a suitable emulsifying agent, a protective colloid and thickener if desired, and an anti-foaming agent to give an emulsion of desired consistency depending upon application requirements. For the above ranges approximately 450 parts of water is preferred.

The film forming component, in the form of an aqueous emulsion or latex, may be any of those substances noted above, although it has been found that cellulose acetate butyrate and ethyl cellulose are more appropriate for solvent type application than for the emulsion type. The adhesion producer can be any of those listed above and the plasticizing and bacteriostatic components include those mentioned for the solution type composition. Appropriate solvents include alcohols as well as the solvents listed above. Satisfactory emulsifying agents are selected from commercially available non-ionic, anionic or cationic surface active agents depending upon the selection of the film former latex and compatibility therewith as well as the ability to form a stable emulsion with the selected adhesive component. The protective colloid added is selected from such substances as methyl cellulose, carboxymethyl cellulose, polyvinyl alcohol, "solubilized" protein, etc., of such grades as will produce the desired viscosity in the completed composition depending upon the requirements of method of application and use.

In preparing a composition of the emulsion type embodying this invention, the latex or film former is usually commercially available as an emulsion. A second emulsion is made by dissolving the adhesion producing component, bacteriostatic agent and plasticizer in the least quantity of volatile solvent which will form a complete solution. It has been found that this usually results in a concentration of approximately 50% nonvolatiles. The emulsifying agent and anti-foaming agent are added to this solution and stirred until well dispersed. With vigorous agitation, sufficient water is added to produce the desired emulsion containing approximately 25% nonvolatiles. As one example of the emulsion type, 200 parts of film former latex are placed into a stainless steel mixing tank and then the 25% adhesion producer emulsion is slowly added thereto with good but not too vigorous agitation. Sufficient water is then added to reduce the nonvolatile content of the mixture to approximately 15% to 25% as desired. Finally sufficient amount of a solution of 3 parts methyl cellulose in 97 parts of cool water is added to produce the desired viscosity and stability. It will be noted that the proportion of volatile solvents used in this composition is purposely kept low to minimize the smarting action of the composition upon first contacting raw flesh.

The degree of inflammability of liquid compositions embodying this invention is also readily controlled. For example, the emulsion type noted above is essentially non-inflammable and a solution type comprising a vinyl copolymer film former, an amine-aldehyde adhesive and a phosphate-ester plasticizer all dissolved in methylene chloride exhibits a very low degree of inflammability.

Either the solution type or the emulsion type of composition will produce upon drying a satisfactory dressing of the character described. The absence or low degree of medication indicates complete safety in the use of such dressing by substantially untrained laymen. The plastic film produced after evaporation of either the volatile solvents or the aqueous emulsion is tough, elastic, transparent, and of controlled adhesiveness to normal skin. The film is water resistant and the extractability

of components thereof by water or body fluids is virtually negligible. Although the composition is sterile and bacteriostatic, it need not include bactericidal agents or other medication.

The liquid compositions produced are stable and non-oxidizing and, if spray application is desired, are of sufficiently low viscosity. Storage problems are minimized since, except as desired to control evaporation of solvent, there is no need for air tight or other pressure type containers for storage. The film, after application, can be peeled away from normal skin without softening or other treatment and without a further application of solvent or water. The film upon application exhibits substantially no adhesiveness for raw flesh and, after drying, no adhesiveness for newly formed skin growing under the dressing so that disturbance of the healing wound or other trauma is virtually non-existent upon removal of the dressing. While the film is water resistant and impermeable to coliform organisms, it is semipermeable to water vapor which might otherwise collect beneath the applied dressing and form either blisters or channels through the dressing to the outside leaving entranceways for obnoxious infection producing material. Accordingly, with the dressing applied, healing therebeneath proceeds under essentially anaerobic conditions. The film formers utilized, when applied according to this invention, produce uniform and substantially bubble-free films free of accidental gas channels or infection admitting openings. Since the dried film is substantially resistant to passage of medicaments therethrough, it may be used to protect selected skin areas from medications desired to be applied only to other areas of the body.

While the compositions and products herein described constitute preferred embodiments of the invention, it is to be understood that the invention is not limited to these precise compositions and products, and that changes may be made therein without departing from the scope of the invention which is defined in the appended claims.

What is claimed is:

1. A liquid dressing for application to skin to provide upon drying an elastic semipermeable self-sustaining peelable film dressing for wounds, burns and incisions, comprising a volatile liquid vehicle for said dressing, a film-former providing upon drying a semipermeable elastic film for controlled outward moisture vapor transmission and substantial impermeability to bacteria and selected from the class consisting of vinyl polymers, including polyacrylic and polymethacrylic ester polymers, cellulose acetate butyrate, ethyl cellulose, and compatible combinations thereof, a synthetic resinous adhesive compatible with said film-former for adhering said film dressing to normal skin but being substantially nonadherent to raw flesh, the cohesive strength of said film dressing being greater than the adhesive strength of said adhesive for peelable removability of said film dressing from skin to which it is applied, and a plasticizer for said film-former and said adhesive effecting in said film dressing controlled flexibility and elasticity thereof for conforming to movements and contours of skin to which it is applied, said film-former and adhesive and plasticizer all being homogeneously admixed in said liquid vehicle for liquid application to skin.

2. A liquid dressing for application to skin to provide upon drying an elastic semipermeable self-sustaining peelable transparent film dressing for wounds, burns and incisions, comprising a latex film-former emulsion providing upon drying a semipermeable elastic film for controlled outward moisture vapor transmission and substantial impermeability to bacteria, a synthetic resinous emulsifiable adhesive compatible with said film-former for adhering said film dressing to normal skin but being substantially nonadherent to raw flesh, the cohesive strength of said film dressing being greater than the adhesive strength of said adhesive for peelable removability of said film dressing from skin to which it is applied, and a

plasticizer for said film-former and said adhesive effecting in said film dressing controlled flexibility and elasticity thereof for conforming to movements and contours of skin to which it is applied, an emulsifying agent for all said components, and water, all said components being uniformly dispersed in water emulsion for liquid application to skin.

3. A liquid dressing for application to skin to provide upon drying an elastic semipermeable self-sustaining peelable transparent film dressing for wounds, burns and incisions, comprising a non-irritating volatile liquid vehicle for said dressing, a synthetic resinous elastomeric film-former providing upon drying a semipermeable elastic film for controlled outward moisture vapor transmission and substantial impermeability to bacteria and selected from the class consisting of vinyl polymers, including polyacrylic and polymethacrylic ester polymers, cellulose acetate butyrate, ethyl cellulose, and compatible combinations thereof, a synthetic resinous adhesive compatible with said film former for adhering said film dressing to normal skin but being substantially nonadherent to raw flesh and selected from the class consisting of glycerol phthalate, abietic-acid-glycerol and organic acid and vinyl modifications thereof, amine aldehyde resins, maleic anhydride modified resins, vinyl modified resins, and compatible combinations thereof, the cohesive strength of said film dressing being greater than adhesive strength of said adhesive for peelable removability of said film dressing from skin to which it is applied, and a plasticizer for said film former and said adhesive effecting in said film dressing controlled flexibility and elasticity thereof for conforming to movements and contours of skin to which it is applied, said film former and adhesive and plasticizer all being homogeneously admixed in said liquid vehicle for liquid application to skin.

4. A liquid dressing for application to skin to provide upon drying an elastic semipermeable self-sustaining peelable transparent film dressing for wounds, burns and incisions, comprising a major proportion of volatile solvent for said dressing, a resin film-former providing upon drying a semipermeable elastic film for controlled outward moisture vapor transmission and substantial impermeability to bacteria and selected from the class consisting of vinyl polymers, including polyacrylic and polymethacrylic ester polymers, cellulose acetate butyrate, ethyl cellulose, and compatible combinations thereof, a synthetic resin adhesive compatible with said film-former for adhering said film dressing to normal skin but being substantially nonadherent to raw flesh, the cohesive strength of said film dressing being greater than adhesive strength of said adhesive for peelable removal of said film dressing from skin to which it is applied, a plasticizer for said film-former and said adhesive effecting in said film dressing controlled flexibility and elasticity thereof for conforming to movements and contours of skin to which it is applied, and a bacteriostatic component for maintaining the sterility of said dressing during storage and use, all said components being homogeneously admixed in said volatile solvent to sprayable consistency for application to skin.

5. A liquid dressing for application to skin to provide upon drying an elastic semipermeable self-sustaining peelable transparent film dressing for wounds, burns and incisions, comprising a non-irritating volatile liquid vehicle for said dressing, approximately 100 parts by weight of a synthetic resinous elastomeric film-former providing upon drying a semipermeable elastic film for controlled outward moisture vapor transmission and substantial impermeability to bacteria and selected from the class consisting of vinyl polymers, including poly-

acrylic and polymethacrylic ester polymers, cellulose acetate butyrate, ethyl cellulose, and compatible combinations thereof, approximately 5 to 80 parts by weight of a synthetic resinous adhesive compatible with said film former for adhering said film dressing to normal skin but being substantially nonadherent to raw flesh and selected from the class consisting of glycerol phthalate, abietic-acid-glycerol and organic acid and vinyl modifications thereof, amine aldehyde resins, maleic anhydride modified resins, vinyl modified resins, and compatible combinations thereof, the cohesive strength of said film dressing being greater than adhesive strength of said adhesive for peelable removability of said film dressing from skin to which it is applied, and up to approximately 80 parts by weight of a plasticizer for said film former and said adhesive effecting in said film dressing controlled flexibility and elasticity thereof for conforming to movements and contours of skin to which it is applied, said film former and adhesive and plasticizer all being homogeneously admixed in said liquid vehicle for liquid application to skin.

6. A liquid dressing for application to skin to provide upon drying an elastic semipermeable self-sustaining peelable transparent film dressing for wounds, burns and incisions, comprising a non-irritating volatile liquid vehicle for said dressing, approximately 100 parts by weight of a synthetic resinous elastomeric film-former providing upon drying a semipermeable elastic film for controlled outward moisture vapor transmission and substantial impermeability to bacteria and selected from the class consisting of vinyl polymers, including polyacrylic and polymethacrylic ester polymers, cellulose acetate butyrate, ethyl cellulose, and compatible combinations thereof, approximately 50 parts by weight of a synthetic resinous adhesive compatible with said film former for adhering said film dressing to normal skin but being substantially nonadherent to raw flesh and selected from the class consisting of glycerol phthalate, abietic-acid-glycerol and organic acid and vinyl modifications thereof, amine aldehyde resins, maleic anhydride modified resins, vinyl modified resins, and compatible combinations thereof, the cohesive strength of said film dressing being greater than adhesive strength of said adhesive for peelable removability of said film dressing from skin to which it is applied, and up to approximately 50 parts by weight of a plasticizer for said film former and said adhesive effecting in said film dressing controlled flexibility and elasticity thereof for conforming to movements and contours of skin to which it is applied, said film former and adhesive and plasticizer all being homogeneously admixed in said liquid vehicle for liquid application to skin.

#### References Cited in the file of this patent

#### UNITED STATES PATENTS

|           |               |               |
|-----------|---------------|---------------|
| 2,231,407 | Castor        | Feb. 11, 1941 |
| 2,415,901 | Nelson et al. | Feb. 18, 1947 |
| 2,456,387 | Cooper        | Dec. 14, 1948 |
| 2,481,419 | Hamilton      | Sept. 6, 1949 |
| 2,563,593 | Engel         | Aug. 7, 1951  |
| 2,580,488 | Vogl          | Jan. 1, 1952  |

#### FOREIGN PATENTS

|         |               |      |
|---------|---------------|------|
| 558,100 | Great Britain | 1943 |
|---------|---------------|------|

#### OTHER REFERENCES

Choy et al.: U. S. Armed Forces Med. J., 3:1241-55, September 1952.

J. A. M. A., Aug. 5, 1944, vol. 125, pp. 969-973, reprint pp. 1-21, "Local Treatment of Thermal Cutaneous Burns," esp. page 15.